

1

2,738,331

## ALKYLTHIO HYDROQUINONES AND MINERAL OIL COMPOSITIONS THEREOF

John W. Brooks, Wenonah, N. J., assignor to Socony Mobil Oil Company, Inc., a corporation of New York

No Drawing. Application March 18, 1952,  
Serial No. 277,300

18 Claims. (Cl. 252—48.2)

This invention relates to alkylthio hydroquinones, to a method for their preparation and to their use as antioxidants in mineral lubricating oils.

It has been known that aromatic mercaptans, such as thiophenol, will react quite readily with quinone to form either phenylthio hydroquinone or phenylthio quinone, depending on whether the thiophenol or the quinone is used in excess in the reaction. As far as is known, however, there has been no disclosure in the art of the formation of alkylthio hydroquinones by the reaction of aliphatic mercaptans with quinone, although some text books indicate generally that mercaptans will react with benzene and naphthoquinones without precisely disclosing the products. In trying the reaction between n-butyl mercaptan and quinone, however, applicant found that when an excess of quinone was employed, a mixture of mono- and di-n-butylthio quinones was formed. On the other hand, when an excess of n-butyl mercaptan was used, a considerable portion of the butyl mercaptan appeared to be oxidized to the disulfide and only a very small amount of n-butylthio-hydroquinone was formed. The present invention, however, provides a method for conducting the reaction between an aliphatic mercaptan, such as n-butyl mercaptan, and quinone whereby alkylthio hydroquinones are obtained in good yield. The method of the invention is applicable even to tertiary alkyl mercaptans, which, as is well known, are more resistant to reactions involving a cleavage of the hydrogen atom from the sulfur atom than the normal and secondary alkyl mercaptans.

The principle of the invention is applicable to aliphatic mercaptans in general and particularly to those having from 1 to about 20 carbon atoms. As non-limiting examples of such mercaptans, the following may be mentioned:

(1) Primary, normal, mercaptans, such as methyl mercaptan, ethyl, propyl, butyl, pentyl, hexadecyl, octyl, decyl, dodecyl, tetradecyl and octadecyl mercaptans;

(2) Secondary mercaptans, such as S-butyl mercaptan, S-octyl mercaptan, S-dodecyl mercaptan and S-octadecyl mercaptan; and

(3) Tertiary mercaptans, such as t-butyl mercaptan, t-octyl mercaptan and t-dodecyl mercaptan.

As far as is known, there has been no disclosure in the prior art of the successful preparation of a tertiary alkylthio hydroquinone. Such compounds prepared by applicant in accordance with the method herein disclosed are, therefore, believed to be new compositions of matter.

2

It is well known that mineral lubricating oils are subject to oxidative deterioration in use, particularly under the conditions of high temperature and pressure encountered by the oils in internal combustion engines and that said oils need to be fortified against such deterioration by the addition thereto of chemical agents, called antioxidants; which are capable of inhibiting oxidation of the oil in use. The alkylthio hydroquinones of the present invention have been found to be excellent antioxidants for this purpose. The present invention, therefore, contemplates the use of these compounds in lubricating oil compositions. Accordingly, the objects of this invention include, first, a method for forming the alkylthio hydroquinones by the reaction of aliphatic mercaptans with quinones. Second, the preparation of a new class of alkylthio hydroquinones, i. e., the tertiary alkylthio hydroquinones. And, third, the provision of lubricating oil compositions containing alkylthio hydroquinones as antioxidants.

20 In accordance with the invention, it has been found that the alkylthio hydroquinones can be prepared in good yield by the reaction of the mercaptan with the quinone in the presence of an acidic catalyst. Suitable acid catalysts are, for example, hydrogen chloride, p-toluenesulfonic acid, sulfuric acid, phosphoric acid, trichloroacetic acid, hydrofluoric acid, etc. A Friedel-Crafts catalyst, such as  $\text{FeCl}_3$ ,  $\text{AlCl}_3$  or  $\text{ZnCl}_2$ , may also be used. It has been found further that the reaction proceeds best at relatively low temperatures, i. e., from about 0° C. to about 100° C., the higher temperatures within this range favoring the formation of the mono-substituted alkylthio hydroquinones and the lower temperatures, i. e., from about 0° C. to about 10-15° C., favoring the formation of the higher-substituted alkylthio hydroquinones (see Examples 7 and 8, Table II). It has been found further that for the desired products to be obtained in good yield, an excess of mercaptan should be used. Although equimolar quantities of quinone and mercaptan may be used in the reaction, it has been found that the use of at least about 2 mols of mercaptan per mol of quinone provides higher yields of the desired alkylthio hydroquinones. The reaction is generally completed in from about 3 to about 6 hours.

45 The method of forming the alkylthio hydroquinones in accordance with the invention is illustrated by the results shown in Tables I and II for a number of reactions carried out between aliphatic mercaptans and hydroquinone. Table I shows the results obtained using HCl as a catalyst. All of these reactions were run under approximately the following conditions. One mol of quinone, about 3 mols of mercaptan and 1200 g. of benzene were stirred at 5-10° C. for 3 to 4 hours while anhydrous HCl was bubbled through. The reaction mixtures were stored over night in a refrigerator and then filtered. The filtrates were washed with water, topped to 125° C. pot temperature to remove benzene and water, and finally topped to 125° C. pot temperature at 0.5 mm. The product from t-dodecyl mercaptan was topped to 150° C. at 0.5 mm. The residues (products) are mainly mixtures of mono-, di- and tri-substituted alkylthio hydroquinones.

TABLE I  
*Reaction of alkyl mercaptans with quinone in the presence  
 of anhydrous HCl*

| Example Number | Reactants                                                                              | Yield |                                                   | Analyses                      |            |                             |            |                 |                                     | Description of Product |  |
|----------------|----------------------------------------------------------------------------------------|-------|---------------------------------------------------|-------------------------------|------------|-----------------------------|------------|-----------------|-------------------------------------|------------------------|--|
|                |                                                                                        | Grams | Percent of Calcd. <sup>2</sup> (Based on Quinone) | Sulfur Analyses (Wt. Percent) |            | Wt. Percent Active Hydrogen |            | Hydroxyl Number |                                     |                        |  |
|                |                                                                                        |       |                                                   | Observed                      | Calculated | Observed                    | Calculated | Observed        | Calculated                          |                        |  |
| 1              | 1108 g. (1 mol) quinone<br>270 g. (3 mols) n-butyl mercaptan<br>1,200 g. benzene       | 122   | 96                                                | 25.2 { 5 25.65<br>4 22.35     | 0.337      | 6 0.54<br>4 0.70            | 285        | 5 300<br>4 392  | Reddish liquid.                     |                        |  |
| 2              | 108 g. (1 mol) quinone<br>270 g. (3 mols) t-butyl mercaptan<br>1,200 g. benzene        | 126   | 73                                                | 19.1 { 4 22.35<br>3 16.16     | 0.722      | 4 0.70<br>3 1.01            | 482        | 4 392<br>3 566  | Light brown liquid                  |                        |  |
| 3              | 81 g. (3/4 mol) quinone<br>292 g. (2 mols) t-octyl mercaptan<br>700 g. benzene         | 105   | 66                                                | 15.2 { 4 16.08<br>3 12.6      | 0.73       | 4 0.50<br>3 0.80            | 334        | 4 281<br>3 442  | Light brown liquid (viscous).       |                        |  |
| 4              | 135 g. (1 1/2 mols) quinone<br>606 g. (3 mols) t-dodecyl mercaptan<br>1,600 g. benzene | 198   | 69                                                | 12.9 { 4 12.54                | 0.389      | 4 0.39                      | 320        | 4 220           | Reddish brown liquid (very viscous) |                        |  |
| 5              | 54 g. (0.5 mol) quinone<br>135 g. (1.5 mols) t-butyl mercaptan<br>600 g. benzene       | 13    | 14                                                | 17.46 { 4 22.35<br>3 16.16    |            |                             |            |                 | Black tarry solid.                  |                        |  |

<sup>1</sup> No HCl catalyst used in this run.

<sup>2</sup> Calculations are based on the assumption that the product is a mixture of the indicated substituted hydroquinones in the proportion indicated by the sulfur analysis. The theoretical amounts of substituted hydroquinones which may result from 1 mol of quinone are: (1) 1 mol of mono-substituted hydroquinone, (2)  $\frac{1}{2}$  mol of di-substituted hydroquinone or (3)  $\frac{1}{4}$  mol of tri-substituted hydroquinone.

### <sup>2</sup> Calculations for mono-alkylthio hydroquinones

#### 4 Calculations for di-alkylthio hydroquinones.

## 5 Calculations for tri-alkylthio hydroquinones

Table II summarizes the results ob-

Table II summarizes the results of

Table II summarizes the results obtained by reacting t-mercaptans with quinone in the presence of p-toluenesulfonic acid under the conditions shown in the table, except that Examples 5 and 6 were run in the absence of the catalyst. It will be seen from Table II that the presence of the p-toluenesulfonic acid catalyst provides markedly improved yields of the alkylthio hydroquinone product, either at low temperature (compare Examples 5 and 7) or at the relatively high temperatures (compare Example 6 with Examples 8-11). In Examples 7 and 8, the quinone, t-butyl mercaptan, benzene and p-toluenesulfonic acid were placed in the flask together and reacted at 10° C. and 80° C., respectively, for 4 hours, while in Examples 9, 10 and 11, the quinone was added to a mixture of the mercaptan, benzene and p-toluenesulfonic acid over a period of about 1½ hours and then the mixture was heated at 80° C. for 4 hours. This latter procedure affords better control of the reaction, which is exothermic, and also insures a good excess of mercaptan at all times in the course of the reaction.

the quinone, t-butyl mercaptan, benzene and p-toluenesulfonic acid were placed in the flask together and reacted at 10° C. and 80° C., respectively, for 4 hours, while in Examples 9, 10 and 11, the quinone was added to a mixture of the mercaptan, benzene and p-toluenesulfonic acid over a period of about 1½ hours and then the mixture was heated at 80° C. for 4 hours. This latter procedure affords better control of the reaction, which is exothermic, and also insures a good excess of mercaptan at all times in the course of the reaction.

TABLE II  
*Reaction of tert-mercaptans with quinone in the presence  
 of p-toluenesulfonic acid*

| Example Number | Reactants                                                                                         | Catalyst                      | Reaction Conditions                                    | Yield |                                         | Analyses                |                   |                   | Description of Product                |
|----------------|---------------------------------------------------------------------------------------------------|-------------------------------|--------------------------------------------------------|-------|-----------------------------------------|-------------------------|-------------------|-------------------|---------------------------------------|
|                |                                                                                                   |                               |                                                        | Grams | Percent of Calcd.<br>(Based on Quinone) | Sulfur (Wt. Percent)    | Molecular Weight  | Hydroxyl Number   |                                       |
| 5.....         | 54 g. (0.5 mol) quinone.....<br>135 g. (1.5 mols) t-butyl mercaptan.....<br>600 g. benzene.....   | None.....                     | 5 hrs. at 5-10° C.....<br>Overnight in refrigerator.   | 13    | 14                                      | 17.46                   |                   |                   | Black tar-like material.              |
| 6.....         | 54 g. (0.5 mol) quinone.....<br>135 g. (1.5 mols) t-butyl mercaptan.....<br>600 g. benzene.....   | do.....                       | 5 hrs. at 50° C.....<br>Overnight at room temperature. | 25    | 28                                      | 18.33                   |                   |                   | Do.                                   |
| 7.....         | 54 g. (0.5 mol) quinone.....<br>135 g. (1.5 mols) t-butyl mercaptan.....<br>600 g. benzene.....   | 15 g. p-toluenesulfonic acid. | 4 hrs. at 10° C.....<br>Over weekend in refrigerator.  | 55    | 70                                      | 20.79<br>16.16<br>22.35 | 226<br>198<br>286 | 373<br>566<br>392 | White solid.                          |
| 8.....         | 54 g. (0.5 mol) quinone.....<br>135 g. (1.5 mols) t-butyl mercaptan.....<br>600 g. benzene.....   | do.....                       | 4 hrs at 80° C.....                                    | 107   | 108                                     | 16.29                   | 192               | 625               |                                       |
| 9.....         | 216 g. (2 mols) quinone.....<br>360 g. (4 mols) t-butyl mercaptan.....<br>2000 g. benzene.....    | 20 g. p-toluenesulfonic acid. | do.....                                                | 326   | 85                                      | 16.92                   | 198               | 560               | White solid.                          |
| 10.....        | 54 g. (0.5 mol) quinone.....<br>146 g. (1 mol) t-octyl mercaptan.....<br>600 g. benzene.....      | 10 g. p-toluenesulfonic acid. | do.....                                                | 112   | 93                                      | 13.35<br>12.6<br>10.08  | 259<br>252<br>398 | 439<br>444<br>281 | Light brown viscous liquid.           |
| 11.....        | 54 g. (0.5 mol) quinone.....<br>303 g. (1.5 mols) t-dodecyl mercaptan.....<br>600 g. benzene..... | do.....                       | do.....                                                | 115   | (?)                                     | 12.82<br>10.3<br>12.53  | 356<br>362<br>220 | 356<br>362<br>220 | Reddish-brown liquid. (Very viscous.) |

<sup>1</sup> Calculations are based on the products being mixtures of mono- and di-substituted alkylthio hydroquinones. The compositions of these mixtures are based on their sulfur analyses. The theoretical amounts of substituted hydroquinones which may result from one mol of quinone are: (1) 1 mol of monalkylthio hydroquinone and (2)  $\frac{1}{2}$  mol of dialkylthio hydroquinone.

<sup>2</sup> The sulfur content of this product is too high. It probably contained some unreacted mercaptan.

<sup>3</sup> Calculations for mono-alkylthio hydroquinones.

\* Calculations for di-alkylthio hydroquinones.

## ANTIOXIDANT ACTION

The products obtained in the reactions described in Tables I and II were blended with oil and the blends were subjected to a modified German tar test to determine the antioxidant properties of the compounds. This test involves heating a 150-gram sample of the oil at a temperature of 120° C. while bubbling oxygen gas through the oil for a period of 70 hours. The acidic oxidation products formed are then determined by titrating with alcoholic potassium hydroxide. Results for the oil alone and for the oil blends are given in Table III in terms of neutralization numbers (N. N.), such numbers representing the acidity of the oil at the end of the test.

The base oil used in this test was a highly refined oil, suitable for use in transformers, which had been prepared by treating a coastal distillate with 40 pounds of 98% sulfuric acid and 180 pounds of 103% oleum per barrel, followed by a clay percolation. It had a specific gravity of 0.871, a flash point of 310 F., and a Saybolt Universal Viscosity of 69 seconds at 100° F. Such an oil forms mainly acidic products on oxidation, which are indicated by a high N. N. value.

TABLE III

| Compound Added | Percent Used | N. N. Value |
|----------------|--------------|-------------|
| None           |              | 18          |
| Example 1      | 0.1          | 0.02        |
| Example 2      | 0.1          | 0.02        |
| Example 3      | 0.1          | 0.02        |
| Example 4      | 0.1          | 0.02        |
| Example 7      | 0.1          | 0.02        |
| Example 8      | 0.1          | 0.02        |
| Example 9      | 0.1          | 0.02        |
| Example 10     | 0.1          | 0.02        |
| Example 11     | 0.1          | 0.02        |

These compounds were also blended with a motor oil to determine their effect on bearing corrosion. Motor oils, especially those refined by certain solvent-extraction methods, tend to oxidize when submitted to high temperatures and form products that are corrosive to metal bearings. This corrosive action may be quite severe with certain bearings, such as those having the corrosion susceptibility of cadmium-silver alloys; and it may cause their failure within a comparatively short time. The following test was used to determine the corrosive action of a motor oil on an automobile connecting-rod bearing.

The oil used consisted of Pennsylvania neutral and residuum stocks separately refined by means of Chlorex, and then blended to give an SAE 20 motor oil with a specific gravity of 0.872, a flash point of 435° F., and a Saybolt Universal Viscosity of 318 seconds at 100° F. The oil was tested by immersing therein about a 6-gram section of a bearing containing a cadmium-silver alloy surface and heating it to 175° C. for 22 hours while a stream of air was bubbled against the surface of the bearing at the rate of two liters per hour. The loss in weight of the bearing during this treatment measures the amount of corrosion that has taken place. The results obtained from this test are given in Table IV.

TABLE IV

| Compound Added | Percent Used | Mg Loss in Wt. |
|----------------|--------------|----------------|
| None           |              | 20             |
| Example 1      | 0.1          | 0              |
| Example 2      | 0.1          | 0              |
| Example 3      | 0.1          | 0              |
| Example 4      | 0.1          | 0              |
| Example 7      | 0.1          | 0              |
| Example 8      | 0.1          | 0              |
| Example 9      | 0.1          | 0              |
| Example 10     | 0.1          | 0              |
| Example 11     | 0.1          | 0              |

Several of the product compounds were also subject-

ed to the Lauson Oxidation Stability Test, the purpose of which is to determine oil deterioration as primarily indicated by corrosion of copper-lead bearings. The oil employed for this test consisted of Pennsylvania neutral and residuum stocks separately refined by means of Chlorex and then blended to give an SAE 10 motor oil. A Lauson single cylinder, 4-cycle, liquid cooled gasoline engine with splash lubrication using copper-lead bearings was operated under the following conditions.

- 10 (1) Oil temperature=270° F.
- (2) Jacket temperature=212° F.
- (3) Speed=1825 R. P. M.
- (4) One-half throttle
- (5) 13:1 air:fuel ratio
- (6) Oil added every 20 hours.

The bearing corrosion results after one hundred hours of operation are shown in Table V.

TABLE V

| Compound Added | Concn. (Wt. Per cent) | Bearing Wt. Loss (G.) Av. of Top and Bottom |
|----------------|-----------------------|---------------------------------------------|
| None           |                       | 0.510                                       |
| Example 1      | 0.5                   | 0.108                                       |
| Example 2      | 0.5                   | 0.053                                       |
| Example 3      | 0.5                   | 0.065                                       |
| Example 4      | 1.0                   | 0.002                                       |
| Example 4      | 0.5                   | 0.081                                       |

From the foregoing test results, it can be observed that the reaction products contemplated herein are highly effective for stabilizing viscous petroleum oil fractions against the normal deteriorating effects of oxidation.

The alkylthio hydroquinones of the invention may be used in the lubricating oil in amounts ranging from about 0.01 per cent up to about 10 per cent, depending upon the particular oil and the amount of improvement desired. For most purposes, however, the use of from about 0.1 to about 2 per cent of the additive is sufficient to provide the desired improvement.

The products herein described may be used in lubricating oils in combination with other addition agents designed to impart different improving properties to the oil, such as detergents, V. I. improvers, pour point depressants, antifoam agents, antirust agents, extreme pressure agents, etc.

Although the invention has been illustrated herein by means of certain specific examples, it is not intended that the scope of the invention be limited thereby, but only as indicated in the following claims.

What is claimed is:

1. A method for preparing an alkylthio-substituted hydroquinone which comprises reacting 1 mol of quinone with at least 1 mol of an aliphatic mercaptan in the presence of an acidic catalyst at a temperature of from about 0° C. to about 100° C. and for a time period of at least about 4 hours.
2. A method for preparing an alkylthio-substituted hydroquinone which comprises reacting 1 mol of quinone with at least 1 mol of an aliphatic mercaptan in the presence of hydrogen chloride at a temperature of from about 0° C. to about 100° C. and for a time period of at least about 4 hours.
3. A method for preparing an alkylthio-substituted hydroquinone which comprises reacting 1 mol of quinone with at least 1 mol of an aliphatic mercaptan in the presence of p-toluenesulfonic acid at a temperature of from about 0° C. to about 100° C. and for a time period of at least about 4 hours.
4. A method for preparing n-butylthio-substituted hydroquinone which comprises reacting 1 mol of quinone with at least about 2 mols of butyl mercaptan in the presence of a paratoluene sulfonic acid at a temperature of from about 0° C. to about 100° C. and for a time period of at least about 4 hours.

5. A method for preparing a t-alkylthio-substituted hydroquinone which comprises reacting 1 mol of quinone with at least about 2 mols of a tertiary aliphatic mercaptan in the presence of paratoluene sulfonic acid at a temperature of from about 0° C. to about 100° C. and for a time period of at least about 4 hours. 7
6. A method for preparing a t-butylthio-substituted hydroquinone which comprises reacting 1 mol of quinone with at least about 2 mols of tertiary butyl mercaptan in the presence of p-toluene sulfonic acid at a temperature of from about 0° C. to about 100° C. and for a time period of at least about 4 hours. 10
7. A method for preparing t-octylthio-substituted hydroquinone which comprises reacting 1 mol of quinone with at least about 2 mols of t-octyl mercaptan in the presence of p-toluene sulfonic acid at a temperature of from about 0° C. to about 100° C. and for a time period of at least 4 hours. 15
8. A method for preparing tertiary dodecylthio-substituted hydroquinone which comprises reacting 1 mol of quinone with at least about 2 mols of tertiary dodecyl mercaptan in the presence of paratoluene sulfonic acid at a temperature of from about 0° C. to about 100° C. and for a time period of at least about 4 hours. 20
9. As a new composition of matter, a tertiary alkylthio-substituted hydroquinone. 25
10. As a new composition of matter, a t-butylthio-substituted hydroquinone.
11. As a new composition of matter, a t-octylthio-substituted hydroquinone. 30
12. As a new composition of matter, a t-dodecylthio-substituted hydroquinone.
13. A mineral lubricating oil containing a minor proportion, sufficient to inhibit said oil against oxidation, of an alkylthio-substituted hydroquinone.
14. A mineral lubricating oil containing a minor proportion, sufficient to inhibit said oil against oxidation, of a n-butylthio-substituted hydroquinone.
15. A mineral lubricating oil containing a minor proportion, sufficient to inhibit said oil against oxidation, of a tertiary alkylthio-substituted hydroquinone.
16. A mineral lubricating oil containing a minor proportion, sufficient to inhibit said oil against oxidation, of a t-butylthio-substituted hydroquinone.
17. A mineral lubricating oil containing a minor proportion, sufficient to inhibit said oil against oxidation, of a t-octylthio-substituted hydroquinone.
18. A mineral lubricating oil containing a minor proportion, sufficient to inhibit said oil against oxidation, of a t-dodecylthio-substituted hydroquinone.

## References Cited in the file of this patent

## UNITED STATES PATENTS

- 2,549,118 Newby \_\_\_\_\_ Apr. 17, 1951  
 2,553,417 Ladd et al. \_\_\_\_\_ May 15, 1951

## OTHER REFERENCES

Recsei, Berichte 60, 1836 (1927).